

# UNITED STATES PATENT OFFICE.

EDWIN J. WATSON AND CHARLES S. HALL, OF WORCESTER, MASS.

## PROCESS OF MANUFACTURING WIRE.

SPECIFICATION forming part of Letters Patent No. 279,295, dated June 12, 1883.

Application filed May 4, 1882. (No model.)

*To all whom it may concern:*

Be it known that we, EDWIN J. WATSON and CHAS. S. HALL, both of the city and county of Worcester, and State of Massachusetts, have invented certain new and useful Improvements in the Method or Process of Manufacturing Wire, of which improvements the following specification is a full description.

This invention has reference to the manufacture of wire by annealing and reducing by means of dies; and its object is to facilitate and improve the annealing and drawing of the wire and to effect a saving of time and expense in the manufacture.

In the ordinary processes of annealing in an annealing pot or muffle, the wire, being exposed hot to the atmosphere, has formed upon its surface a scale or coating of oxide of iron. If this scale were allowed to remain, it would in the process of drawing cut and otherwise injure the dies and interfere with their operation, and the wire produced would be of a very inferior quality. The removal of such scale before drawing the wire is therefore imperative, and it is commonly effected by treatment in an acid bath. This treatment, however, renders the wire brittle and necessitates frequent annealing to soften the wire during the drawing process. It also necessitates other treatment—such as "bluing"—to remove the ill effects of the acid, in course of which the liability to the formation of a new scale is incurred. These frequent cleanings and reannealings render production of wire very tedious and costly. When the annealing is performed, as is sometimes done, by immersing the wire rods or stock in a bath of melted lead, instead of a scale of oxide of iron being formed thereon, it becomes coated with a layer of lead oxide; but this has always been considered objectionable, and no matter what the nature of the crust formed incidental to the process of annealing, it has been the invariable practice heretofore to remove it, either by treatment with acids or by cleaning or scouring in some other way, before drawing the wire through dies.

Our invention consists in annealing the wire rods in melted lead, as above indicated, thus forming a layer of lead oxide thereon, and then wire-drawing without removing such layer, we having found that the presence of the coat-

ing of lead oxide, in connection with a coating of lime, flour, meal, or other known or suitable lubricant, or anti-friction material, 55 enables the wire to be more freely and easily drawn through dies, and with less frequent softening than has been possible under the processes in common use.

In order that our invention may be the better understood by persons skilled in the art to which it relates, the manner in which the same is or may be carried into effect will now be described more in detail.

The wire rods or wire as taken off the reel 65 in the rolling-mill are dipped in bulk in a bath of melted lead, so as to be in direct contact with the fused metal therein. The heat of the bath and the length of continuance of the treatment will be varied, as well understood, according to the nature of the material dealt with and the character of final product desired. The heat of the bath can be very nicely regulated to avoid overheating or imperfect annealing from insufficient heat. The stock 70 under treatment in the bath can be quickly changed and heat economized by keeping the latter at or near the same temperature. When the rods or wire are removed from the bath they are coated with lead oxide. This coating 75 prevents scaling, and, moreover, by allowing it to remain on the wire in the process of drawing, that operation, instead of being hindered, will be greatly facilitated. Instead, therefore, of cleaning off the coating by acids 80 or otherwise, as in the ordinary processes of manufacture, it is retained on the rods. These are next coated with lime, flour, meal, or other known or suitable lubricant or anti-friction coating, and four drafts may be drawn through 85 the dies, reducing the wire to No. 12 without reannealing, we having found by experiment that the presence of the coating of lead oxide enables more drafts to be drawn without reannealing than could otherwise be done. The 90 No. 12 wire is then reannealed, as before, in melted lead, a new coating of lead oxide being thus formed, and the wire again coated with lime, flour, meal, or other lubricant, when it 95 may be drawn to No. 15.

It will be seen that by the new process of drawing wire the time of the operation is greatly shortened, and that it will enable manufacturers to largely increase their production.

With the presence of the coating of lead oxide, not only is the drawing through dies facilitated, but the wire produced is of an exceedingly fine quality, very strong, and uniform 5 in texture.

A very great saving is effected by dispensing with the frequent cleanings in acid after annealing, which heretofore has ordinarily been necessary three or more times during the 10 drawing of the wire. The acid treatment, moreover, affected the character of the wire itself, rendering it brittle and necessitating frequent reannealing. These objections and difficulties are also removed by the present improvement. 15

When the wires have become rusty, or have been annealed otherwise than by the process indicated, or when for any other reason it has been necessary to clean them in acid, the treatment 20 in a lead bath may be advantageously substituted for the ordinary process of bluing, or heating to about a blue heat to remove the effects of the acid.

We have referred to melted lead solely in 25 the foregoing description; but any other metal or metallic alloy which will accomplish the purposes may be used—as, for example, tin, antimony, or alloys of the same or of lead, and our invention includes the use of such.

In the process of wire-drawing any known 30 or suitable lubricant or anti-friction material other than those indicated may be employed.

Having now fully described our said invention and the manner in which the same is or may be carried into effect, what we claim, and 35 desire to secure by Letters Patent, is—

1. As an improvement in the art of manufacturing wire, the method of annealing the wire rods in a bath of melted lead in direct contact with the melted metal, whereby a coating of lead oxide is formed on said wire rods, and drawing the same through dies with the coating of lead oxide thereon, substantially as 40 described.

2. The method of manufacturing wire by 45 forming on the wire rods or stock a coating of lead oxide, as by annealing in a bath of melted lead, then coating with lime, flour, meal, or other anti-friction coating, and wire-drawing through dies, substantially as described.

EDWIN J. WATSON.  
CHARLES S. HALL.

Witnesses:

JOHN C. DEWEY,  
THOS. H. DODGE.